

## UNITED STATES PATENT OFFICE.

WILLIAM HARRISON, OF MANCHESTER, ENGLAND.

## MANUFACTURE OF WOOL-LIKE CELLULOSIC MATERIAL.

No Drawing. Application filed January 26, 1927, Serial No. 163,851, and in Great Britain February 12, 1926.

This invention relates to the manufacture of wool-like cellulosic material.

The object of this invention is to produce a material from a cellulosic fibre which has 5 more of the properties of wool in relation to elasticity, warmth and shrinking properties than materials produced by hitherto known processes and which at the same time will possess the necessary stability to retain 10 its properties.

It is known that cotton, and particularly unbleached cotton when treated with nitric acid of certain concentration acquires some 15 of the characteristics of wool and also that sulphuric acid under certain conditions produces a similar effect but neither of the processes gives a material which can be shrunk except by treatment with caustic soda of a concentration of over 12%. Furthermore 20 neither process is easy to carry out in practice because of the known tendering action of acids on cellulose and neither process produces a product having any great similarity to wool.

25 It is also known that by subjecting a cellulosic material such as cotton either with or without the application of tension to the combined action of caustic soda and carbon disulphide, a xanthate can be produced 30 which is insoluble in water but which like the soluble xanthate known as viscose is very unstable. It is readily decomposed by dilute solutions of mineral acids, by strong oxidizing agents such as hypochlorites, by heat 35 and also spontaneously when in contact with water or alkaline solutions. For example, during the drying of materials containing or consisting of this insoluble xanthate by the customary methods used in the textile industry decomposition takes place and the 40 material acquires a yellow color from the by-products formed.

The production of this unstable and insoluble xanthate has been described in a 45 number of previous patents e. g.—Ashwell, British Patent No. 19,012 of 1901; Cross & Bevan, British Patent No. 126,174; Lilienfeld, British Patent No. 216,476; Lilienfeld, British Patent No. 216,477; Aykroyd & 50 Hrais, German Patent No. 6850/1899 and Joliot, German Patent No. 322,047.

On account however of the instability of the product it has not hitherto been found possible to use it commercially.

I have discovered, that this unstable insoluble xanthate can be formed into a stable compound which is more wool-like than the unstable compound, and which moreover will maintain its wool-like properties.

According to the invention the unstable insoluble xanthate is subjected to the action of a mild oxidizing agent which will not completely split off the carbon disulphide already combined with the cellulose to convert it into a compound which will not be 60 decomposed by dilute solutions of mineral acids, by heat or by long standing in contact with water and which being reactive imparts shrinking properties to the cellulosic material.

In carrying out the invention a cellulosic fibre such as cotton, either with or without the application of tension at any stage during the process, is subjected to the combined action of caustic alkalies or alkaline sulphides or mixtures of the same and carbon disulphide. The amount of carbon disulphide and the time of treatment are so arranged that the product obtained is insoluble or only sparingly or partially soluble in 80 water. The carbon disulphide may be applied in vapour form or in solution in an inert solvent such as benzene, either before or after, but preferably after treatment with the alkaline solution or may be applied simultaneously with the alkaline solution in the form of an emulsion suspension or colloidal solution in the alkaline solution. The caustic soda may also be applied both before and after the treatment with carbon 85 disulphide and the material may or may not be subjected to tension during either or both of these treatments with caustic soda or of subsequent washing. By application of tension particularly during the washing process 90 a lustre similar to that of wool may be imparted.

Generally speaking the amount of carbon disulphide and/or the time of treatment are to be raised in an inverse ratio to the 100 concentration and/or amount of alkaline solution applied to the cellulosic fibre.

The unstable insoluble xanthate produced by the above process or by any other process is then washed with water or with salt 105 solution to remove the by-products, this washing process being performed rapidly so as to prevent appreciable decomposition

of the xanthate and the material is then, while it is or is not subjected to tension or after acidifying with a weak acid such as acetic acid, subjected to the action of a 5 mild oxidizing agent such as oxygen, or atmospheric air,—preferably in presence of a suitable catalyst such as the oxides of iron, cobalt, nickel or manganese,—ferricyanides, iodine, nitrous acid and other oxides of 10 nitrogen and any other mild oxidizing agent which does not completely split off the carbon disulphide already combined with the cellulose.

Of these mild oxidizing agents nitrous 15 acid lends itself admirably to the process since it is much cheaper than ferricyanides or iodine and its action is considerably more rapid than air even in presence of catalysts. The nitrogen oxides formed in the reaction 20 may colour the cellulosic material but this colour is readily removed by means of sulphurous acid.

By reason of this mild oxidizing process 25 the unstable xanthate is converted into another compound, most probably by the union of two of the carbon disulphide residues, which is not decomposed by dilute solutions of mineral acids nor by heat nor by long standing in contact with water and 30 which being reactive imparts shrinking properties to the cellulosic material.

The following example, to which it is to be understood that the invention is in no way limited illustrates how the process 35 may be carried out:—

Unbleached cotton preferably in the form 40 of yarn is impregnated with caustic soda of 15% strength the excess being removed in a hydroextractor. The impregnated yarn is then placed in a closed chamber and subjected to the action of carbondisulphide in 45 vapour form and 15% of the weight of the cellulose for a period depending on the amount of carbon disulphide used usually less than four hours.

The insoluble xanthate formed is washed 50 free from the yellow by-products with water and treated with a solution of nitrous acid preferably with addition of acetic acid until 55 the evolution of gaseous by-products ceases. The stable compound formed usually becomes coloured by this process but can be decolourized by means of sulphurous acid.

The final product is then dried either before 60 or after bleaching in the usual way and thereby acquires wool-like properties.

Fibres, yarns or fabrics treated by this 65 process of insoluble xanthogenation followed by mild oxidation are much more elastic than cotton, have greater warmth and can readily be shrunk and the extent to which these properties can be imparted can be varied within extremely wide limits by varying the conditions of treatment at the several 70 stages in the process.

The new products have dyeing properties very different from those of ordinary cellulosic fibres, having strong affinity for basic colours and for certain acid colours particularly those of the sulphonated basic type. 75

The dyeing and other properties can be modified further by making use of the reactivity of the compounds produced by this process towards many organic compounds particularly those of basic character of 80 which compounds containing one or more basic nitrogen groupings are examples. Aniline benzylamine and phenylhydrazine are particularly reactive and impart affinity for other acid colours. Soluble derivatives 85 of anhydroformaldehyde aniline may also be applied to improve the affinity towards ordinary acid colours of the azo type.

Shrinking of the materials can be produced in a variety of ways such as for example by treating the material with ammonia, sodium sulphide or sodium sulphite preferably in the presence of an alkali or with caustic soda of less than 12% strength with or without the addition of ammonia 90 sodium sulphide or sulphite.

The process may be applied to cellulosic fibers such as cotton, linen, ramie, jute and the like or to cellulosic artificial silks, in the form of fibers, yarns or fabrics but of 95 these, yarns offer advantages in so far that a large variety of new effects can be secured in fabrics by making use of the altered dyeing properties more particularly by using 100 yarns subjected to different degrees of treatment by the process and because the shrinking properties can be utilized to give special properties as regards elasticity, warmth and general handle of the result fabrics.

What I claim as my invention and desire 105 to protect by Letters Patent is:—

1. Process for the production of wool-like cellulosic material consisting in subjecting the unstable insoluble xanthate, formed by the combined action of a caustic alkali or alkaline sulphide or any mixture of these and carbon disulphide on cellulosic material, to the action of a mild oxidizing agent which does not completely split off the carbon disulphide previously combined with the cellulose and which converts the unstable insoluble xanthate into a stable compound. 115

2. Process for the production of wool-like cellulosic material which consists in subjecting the unstable insoluble xanthate, formed by the combined action of a caustic alkali or alkaline sulphide or any mixture of these and carbon disulphide on cellulosic material, to the action of nitrous acid, which converts the unstable insoluble xanthate into a stable compound. 120

3. Process for the production of wool-like cellulosic material which consists in subjecting the unstable insoluble xanthate, 125

formed by the combined action of a caustic alkali or alkaline sulphide or any mixture of these and carbon disulphide on cellulosic material, to the action of nitrous acid and acetic acid, which converts the unstable insoluble xanthate into a stable compound. 5. Wool-like cellulosic material produced by subjecting the unstable insoluble xanthate to the action of nitrous acid.

4. Wool-like cellulosic material produced by subjecting the unstable insoluble xanthate to the action of a mild oxidizing agent. In testimony whereof I have hereunto set my hand.

WILLIAM HARRISON.